

## UNITED STATES PATENT OFFICE

2,580,923

PREVENTION OF CORROSION IN STEAM  
GENERATION

Arthur L. Jacoby, Western Springs, Ill., assignor  
to National Aluminate Corporation, Chicago,  
Ill., a corporation of Delaware

No Drawing. Application June 19, 1947,  
Serial No. 755,739

10 Claims. (Cl. 252—180)

1

This invention relates to the art of treating water in boilers, steam generators, evaporators and the like, and the treatment of the steam and the condensate produced therefrom to reduce or prevent the corrosion of steam lines, traps, condensers and other pieces of equipment carrying the steam and the condensate. The invention also relates to the preparation of new and improved water treating compositions.

It has heretofore been suggested that certain amines may be added to boiler water from which they will volatilize with the steam and condense and dissolve in the condensed steam to inhibit corrosion occurring in the condensate lines. These amines may also be added directly to the steam lines. The amines proposed for this purpose are liquids boiling within the range from 0 degrees C. to 171 degrees C. at atmospheric pressure. These liquid amines are, in general, highly caustic and present a serious hazard in their handling. Furthermore, they are quite volatile even under ordinary temperature conditions and the toxicity of their fumes in high concentrations presents a further hazard in their use. Moreover, the addition of liquids to a boiler or to the steam lines is attended with many mechanical and practical difficulties.

One of the objects of the present invention is to provide a composition for the treatment of boiler water, steam and steam condensates, which composition is in substantially dry form that is readily soluble or dispersible in water, and from which suitable amines are liberated by the action of alkaline boiler water.

Another object of the invention is to prepare corrosion inhibiting compositions of the type described in the form of briquettes which are gradually and uniformly dissolved in the feed water to a steam boiler, evaporator or the like. Other objects will appear hereinafter.

In accomplishing these objects in accordance with the invention it has been found that corrosion inhibiting amines suitable for use in steam generating systems can be prepared in the form of crystalline non-hygroscopic water soluble salts. These amine salts are solids which are capable of liberating the free amines when added to the feed water of a steam boiler containing sufficient alkali to decompose the amine salts into free amines at steam generating temperatures. These solid amine salts can also be incorporated with other water treating chemicals either by mixing them together to produce a dry, free flowing powder or by briquetting them with a suitable binder, preferably one which is water soluble. The preferred compositions consist of the amine salts briquetted with other water treating chemicals, e. g., tannins, lignin sulfonates, sodium sulfite, or the like, by means of binders such as dextrines.

2

Assuming that the alkali added to the boiler water is sodium hydroxide, the general reaction which occurs between the amine salt and the alkali with the liberation of the amine may be described by the following equation:



Generally speaking, the quantities of amine salt required for the purpose of the invention are so small that the quantities of alkali employed in the boiler water will be sufficient to react with the amine salt and liberate the free amine while still maintaining an alkaline condition in the boiler water. In some cases, however, where the amine salt is made up with an excess of acid or acid salt, it may be desirable to add larger amounts of alkali to the boiler feed water to compensate for the alkali which is utilized in the reaction with the amine salt. The quantity of alkali required for this purpose can readily be calculated by any one skilled in the art.

The amines which are useful for the preparation of amine salts in accordance with the practice of the invention are, in general, aliphatic, alicyclic, cycloaliphatic, aromatic, and heterocyclic amines possessing the following properties:

1. The amine should distill or volatilize with steam in appreciable quantities in the boiler pressure range of superatmospheric pressures from 5 to 250 pounds per square inch or at higher pressures if such pressures are employed.

2. The amine should not cause foaming and carryover.

3. It should not decompose appreciably under boiler conditions of alkalinity, pH, pressure and temperature.

4. The boiling point of the amine should preferably be above 100 degrees C. so that appreciable amounts of the amine are not lost in venting or preheating of the feed water and so most of the amine will be in the liquid phase in the portions of the system handling hot condensate. It should be pointed out that boiling point alone

is not the factor which determines the relative volatility of the amine with steam, as the tendency to form stable hydrates and other factors also influence this behavior.

5. The amine should not form stable carbonic acid addition products which will not decompose to the amine and carbon dioxide at preheater temperatures.

6. The carbonic acid addition products of the amine should be reasonably water soluble.

7. The amine should have a low equivalent weight. The lower the weight of the amine for each neutralizing amino group the less the quantity of the amine required to inhibit corrosion in the steam system.

8. The amine should preferably be of a type

which forms a protective film on the steam and condensate lines that will inhibit oxygen corrosion.

9. The amine should preferably have such vapor pressure characteristics that in boiling dilute aqueous solutions little change occurs in the water to amine ratio, thus providing nearly constant alkalinity in the boiling water and the steam condensate.

Specific examples of suitable amines for most steam systems are: morpholine (B. P. 126-130 degrees C.), monoethanolamine (B. P. 171 degrees C.), cyclohexylamine (B. P. 134 degrees C.), benzylamine (B. P. 184 degrees C.) and dimethyl-ethanolamine (B. P. 133.5 degrees C.). These amines are miscible with water in all proportions. Other amines, such as aniline, which is only partially soluble in water, are unsatisfactory for the purpose of the invention. Amines which are soluble in water but have relatively high boiling points, e. g., triethanolamine, which boils around 280 degrees C. under a partial vacuum are not adapted for steam generation under pressures within the preferred range from 5 to 250 pounds per square inch but might be used in steam generation under higher pressures and the corresponding temperatures. It will be observed that the above described amines are illustrative of primary, secondary and tertiary amines.

The amine salts of mineral acids and organic carboxylic and/or sulfonic acids can be prepared by dissolving the acid in a solvent, e. g., water, diethyl ether or methanol, and adding the equivalent quantity of amine with stirring at a rate such as to avoid overheating. Cooling may be resorted to in some cases. The salt is then recovered by filtration and, if necessary, evaporation. In cases where the corresponding amide is water insoluble care must be taken in the preparation of the salt to avoid dehydration to the amide. Another way in which the amine salts may be conveniently prepared consists in conducting the neutralization of the amine in the presence of a solid material capable of absorbing the water of reaction, thereby yielding a dry appearing product without actually drying by evaporation. An example of this procedure is to mix an amine with a large excess of sodium acid sulfate either with or without the addition of anhydrous sodium sulfate. The amine will then be converted to a mixed amine salt, namely, sodium amine sulfate, and the water will be absorbed by the excess of salt or salts producing a dry appearing powder.

The following amine salts or mixed salts have been prepared in accordance with the invention and have been found to be suitable for the practice of the invention:

A. The hydrochloride, the hydrobromide, the nitrate, the sulfate, the orthophosphate, the acetate, the phenyl acetate, and the 2-naphthalene sulfonate of morpholine;

B. The hydrochloride, the hydrobromide, the nitrate, the sulfate, the orthophosphate, the acetate, the phenyl acetate, the pyrophosphate salt of cyclohexylamine and the 2-naphthalene sulfonate of cyclohexylamine;

C. The hydrochloride, the hydrobromide, the orthophosphate, the phenyl acetate, the acid oxalate of monoethanolamine, and the 2-naphthalene sulfonate of monoethanolamine;

D. The nitrate, the sulfate, the orthophosphate, the acetate, the phenyl acetate and the 2-naphthalene sulfonate of benzylamine; and

E. The acid oxalate of dimethylethanolamine. Additionally, mixed alkali metal amine salts

are suitable for the practice of the invention, for example, cyclohexylamine, sodium sulfate (i. e., the sodium ammonium sulfate), the mixed morpholine salts of lignin sulfonic acid and sulfuric acid, morpholine sodium sulfate. In reacting the amines with the alkali metal acid salts, an excess of the acid salt was used and hence the amine groups were neutralized.

The above mentioned amine salts or mixed amine salts are substantially non-hygroscopic solid water soluble salts, but it will be understood that not all amine salts have satisfactory properties for the purpose of the invention even though the amine itself may be suitable in other respects for inhibiting corrosion in a steam system. Thus, the orthophosphate, the metaphosphate, the arsenate, the borate, the sulfite, the benzene sulfonate and the paratoluene sulfonate of morpholine were all found to be too hygroscopic for the purpose of the invention. Similarly, the hydrochloride, the nitrate, the sulfate, the orthophosphate, the acetate, the phenyl acetate and the 2-naphthalene sulfonate of dimethyl-ethanolamine were too hygroscopic to be isolated. The nitrate, the sulfate and the acetate of monoethanolamine were all too hygroscopic.

The following examples are given to show methods of preparing amine salts suitable for the practice of the invention and also to illustrate the preparation of compositions containing such salts, it being understood, however, that these examples are not intended to limit the scope of the invention.

#### Example I

To 87 parts by weight of morpholine was added 85.7 parts by weight of 70% nitric acid. The addition was made with thorough mixing and at a rate such that the temperature was maintained at 105 degrees C. to 110 degrees C. When the addition was complete the temperature was permitted to drop and the mixture became a heavy mass of damp crystals which were useful in that state if mixed with sufficient other water soluble portions of a water treating composition, or were readily dried to a point where they were free flowing by themselves or compatible with other chemicals to give a powdered product containing a greater amine salt content than would be possible in the compositions containing the moist salt.

#### Example II

Morpholine sulfate was prepared in the manner described in Example I except that equivalent amounts of concentrated sulfuric acid were employed instead of the nitric acid. It was found that by keeping the temperature of neutralization at 50° C. or below, the amine salt was much less prone to absorb moisture and gave a better product. The resultant product was a white granular powder of very faint morpholine odor. Similarly, the hydrochloride, the orthophosphate and the hydrobromide of morpholine were prepared using the appropriate acid instead of the nitric acid of Example I.

In a like manner, by substituting equivalent amounts of the amine and/or the acid, the following amine salts were prepared; the nitrate, the sulfate and the orthophosphate of cyclohexylamine; the hydrochloride and the orthophosphate of monoethanolamine; and the sulfate, the nitrate and the orthophosphate of benzylamine.

In the following examples, III to VI, inclusive, the procedure of mixing to add the liquid

amine to the solid components, omitting the binder (dextrin) and water until last. The mixing was conveniently done in a "putty chaser." The materials shown were made into briquettes.

*Example III*

|                            | Parts |
|----------------------------|-------|
| Alkali soluble humic acids | 10    |
| Cyclohexylamine            | 5     |
| Sodium sulfate, anhydr     | 3.5   |
| Ground nitre cake          | 4     |
| Dextrin                    | 2     |
| Water                      | 1     |

*Example IV*

|                                       | Per cent |
|---------------------------------------|----------|
| Morpholine nitrate                    | 65       |
| Monosodium phosphate, anhydr          | 12       |
| Sodium acid pyrophosphate             | 15       |
| Ammonium sulfate                      | 5        |
| Water (trace used during briquetting) | 20       |
| Dextrin                               | 3        |

*Example V*

|                             | Per cent |
|-----------------------------|----------|
| Morpholine nitrate          | 66       |
| Ammonium sulfate            | 5        |
| Chestnut tannin, dry        | 13       |
| Sodium sulfite              | 5        |
| Dextrin                     | 9        |
| Water (used in briquetting) | 2        |

*Example VI*

|                    | Per cent |
|--------------------|----------|
| Morpholine nitrate | 25       |
| Sodium sulfate     | 31       |
| Sodium sulfite     | 31       |
| Dextrin            | 8        |
| Water              | 5        |

*Example VII*

There was first prepared a mixture of morpholine salts of lignin sulfonic acid and sulfuric acid in the following manner. One part of morpholine and 2.2 parts of lignin sulfonic acid (obtained from waste sulfite liquors) were mixed and sufficient dilute sulfuric acid added to bring the pH down to about 4.7. This material was then dried on a drum drier to a moisture content of about 6% to 7%, whereupon it was found to be a dry, water soluble powder. The amine salt formed was mixed morpholine lignin sulfonate and morpholine sulfate.

The above described powder was then compounded, e. g., as follows:

*Example VIII*

|                           | Per cent |
|---------------------------|----------|
| Mixed salt of Example VII | 50       |
| Nitre cake                | 5        |
| Sodium sulfate            | 35       |
| Dextrin                   | 6        |
| Water (for briquetting)   | 4        |

As previously stated, in order to introduce the amine salt into the steam system it is preferable to prepare it in the form of a briquette with other water treating chemicals and to cause it to be dissolved uniformly and gradually by the feed water to the boiler. This is conveniently accomplished by preparing the briquette and introducing it into a by-pass feeder which is connected in the boiler feed water line. The boiler feed water circulates through the feeder, gradually dissolving the briquette and carrying the amine salt into the boiler where the amine is liberated by the action of the heat and inorganic alkali present. The liberated amine is then

preferably volatilized at a uniform rate such that little change occurs in the water to amine ratio. The manner in which the amine volatilizes will, of course, depend upon the chemical and physical characteristics of the amine. The volatilized amine should serve to provide a nearly constant alkalinity in the boiling water and should redissolve in the steam condensate to provide the desired alkalinity in the latter at the point where condensation occurs.

The quantity of the amine salt initially added to the water from which the steam is generated should preferably be approximately 0.015 pound for each neutralizing amino group per grain of methyl orange alkalinity per thousand gallons of water. This means that if the methyl orange alkalinity of the feed water were 10 the quantity of amine salt would be that quantity capable of liberating 0.15 pound of said amine per thousand gallons of feed water. If the methyl orange alkalinity were 20 the recommended dosage of amine salt would be the equivalent of 0.30 pound of said amine per thousand gallons of water. In a similar manner the dosage can be calculated for waters of different alkalinites. These dosages are based upon a pressure of 250 p. s. i. and the corresponding steam temperatures with adequate venting of the preheater.

The dosage can also be established by observation of the pH obtained in the condensate. In general, it is preferable to maintain a pH in the steam condensate of about 7.0, although it has been observed that substantial corrosion protection has been obtained at a lower pH, as low as 6.3. The preferred pH range in the steam condensate is about 6.5 to about 7.5.

The treatment described herein can be employed in steam generation where the steam generators are operated at operating pressures from a high vacuum to rather high super-atmospheric pressures. It will be understood, however, that of the amines suggested some would be better than others for different pressure operations. Thus, for treatments involving vacuum evaporation the amine salts of cyclohexylamine are recommended. For corrosion prevention or inhibition in steam generating systems operating at superatmospheric pressures within the range of 100 to 250 pounds per square inch and the corresponding temperatures (170 degrees C. to 210 degrees C.) excellent results have been obtained with the amine salts of morpholine.

Having thus described the invention, what I claim as new and desire to secure by Letters Patent of the United States is:

1. In a system wherein steam is generated from a boiler water containing an alkali and condensed, the process which comprises introducing into said boiler water containing an alkali a quantity of a substantially non-hygroscopic water soluble salt of a mono-amine miscible with water in all proportions and volatile with steam at the boiler temperatures and pressures, the quantity of alkali in said boiler water being in excess of the amount required to hydrolyze said amine salt to the free amine, and the quantity of amine salt being effective to liberate a corrosion inhibiting quantity of said volatile amine in sufficient amount to produce a pH in the steam condensate of at least 6.3.

2. In a system wherein steam is generated from a boiler water containing an alkali and condensed, the process which comprises introducing into said boiler water containing an alkali a quantity of a substantially non-hygro-

scopie water soluble salt of a mono-amine miscible with water in all proportions and volatile with steam at the boiler temperatures and pressures, the quantity of alkali in said boiler water being in excess of the amount required to hydrolyze said amine salt to the free amine, and the quantity of amine salt being effective to liberate a corrosion inhibiting quantity of said volatile amine in sufficient amount to produce a pH in the steam condensate within the range of about 6.5 to about 7.5.

3. In a system wherein steam is generated from a boiler water containing an alkali and condensed, the process which comprises introducing into said boiler water containing an alkali a quantity of a substantially non-hygroscopic water soluble salt of a mono-amine miscible with water in all proportions and volatile with steam at the boiler temperatures and pressures, the quantity of alkali in said boiler water being in excess of the amount required to hydrolyze said amine salt to the free amine, and the quantity of amine salt corresponding to that quantity capable of liberating approximately 0.015 pound of amine per grain of methyl orange alkalinity per thousand gallons of boiler feed water.

4. In a system wherein steam is generated and condensed the method of protecting metal parts of the system against corrosion which comprises incorporating into boiler feed water, from which the steam is generated, and which contains an alkali, a quantity of a substantially non-hygroscopic morpholine salt, the quantity of alkali in said boiler water being in excess of the amount required to hydrolyze said morpholine salt to free morpholine, and the quantity of morpholine salt being effective to liberate a corrosion inhibiting quantity of morpholine in sufficient amount to produce a pH in the steam condensate of at least 6.3.

5. In a process of generating steam the method which comprises generating steam from an alkaline boiler water at pressures within the range of 100-250 pounds per square inch and the corresponding temperatures while incorporating into the feed water to the boiler a quantity of non-hygroscopic water soluble salt of morpholine, the quantity of alkali in the alkaline boiler water being in excess of the amount required to hydrolyze said morpholine salt and the quantity of the morpholine salt being sufficient to liberate a corrosion inhibiting quantity of morpholine upon said hydrolysis in sufficient amount to produce a pH in the steam condensate of at least 6.3.

6. In a process of generating steam the method which comprises generating steam from an alkaline boiler water at a pressure approximating 250 pounds per square inch, and the corresponding temperature while incorporating with the boiler feed water a quantity of a water soluble substantially non-hygroscopic morpholine salt capable of liberating approximately 0.015 pound of morpholine per grain of methyl orange alkalinity per thousand gallons of boiler feed water, the quantity of alkali in said boiler water being in excess of the amount required to hydrolyze said morpholine salt, and the quantity of morpholine salt being sufficient to maintain a pH in the steam condensate within the range of about 6.5 to 7.5.

7. In a process of generating steam the method which comprises generating steam from an alkaline boiler water at pressures within the range of 100 to 250 pounds per square inch, and the corresponding temperatures, while incorporating

into the boiler feed water a quantity of morpholine nitrate, the quantity of alkali in the alkaline boiler water being in excess of the amount required to hydrolyze said morpholine nitrate, and the quantity of morpholine nitrate being effective to liberate a quantity of morpholine sufficient to produce a pH in the steam condensate within the range of 6.5 to 7.5.

8. In a process of generating steam the method which comprises generating steam from an alkaline boiler water at pressures within the range of 100 to 250 pounds per square inch, and the corresponding temperatures, while incorporating into the boiler feed water a quantity of morpholine sulfate, the quantity of alkali in the alkaline boiler water being in excess of the amount required to hydrolyze said morpholine sulfate, and the quantity of morpholine sulfate being effective to liberate a quantity of morpholine sufficient to produce a pH in the steam condensate within the range of 6.5 to 7.5.

9. In a process of generating steam the method which comprises generating steam from an alkaline boiler water at pressures within the range of 100 to 250 pounds per square inch, and the corresponding temperatures, while incorporating into the boiler feed water a quantity of cyclohexylamine sulfate, the quantity of alkali in the alkaline boiler water being in excess of the amount required to hydrolyze said cyclohexylamine sulfate, and the quantity of cyclohexylamine sulfate being effective to liberate a quantity of cyclohexylamine sufficient to produce a pH in the steam condensate within the range of 6.5 to 7.5.

10. In the process of generating steam the method which comprises generating steam from an alkaline boiler water at pressures within the range of 100 to 250 pounds per square inch, and the corresponding temperatures, while incorporating into the boiler feed water a quantity of a mixed amine salt of morpholine lignin sulfonate and morpholine sulfate, the quantity of alkali in the alkaline boiler water being in excess of the amount required to hydrolyze said mixed amine salt of morpholine lignin sulfonate and morpholine sulfate, and the quantity of mixed amine salt of morpholine lignin sulfonate and morpholine sulfate being effective to liberate a quantity of morpholine sufficient to produce a pH in the steam condensate within the range of 6.5 to 7.5.

55

ARTHUR L. JACOBY.

## REFERENCES CITED

The following references are of record in the file of this patent:

## UNITED STATES PATENTS

| Number    | Name           | Date          |
|-----------|----------------|---------------|
| 1,903,287 | Cox            | Apr. 4, 1933  |
| 2,053,024 | Dreyfus        | Sept. 1, 1936 |
| 2,200,184 | Morgan         | May 7, 1940   |
| 2,220,950 | Bird           | Nov. 12, 1940 |
| 2,274,807 | Rawlins et al. | Mar. 3, 1942  |
| 2,419,327 | Wachter et al. | Apr. 22, 1947 |
| 2,432,839 | Wachter et al. | Dec. 16, 1947 |
| 2,460,259 | Kahler         | Jan. 25, 1949 |

## OTHER REFERENCES

Dictionary of Organic Compounds, Heilbron, Oxford Press, N. Y., vol. 2 (1943), p. 840.